

1

2,893,812

## DYEING OF MIXED TEXTILE MATERIALS

Yves Henri Guyonnet, Villefranche-sur-Saône (Rhône), France, assignor to Société Rhodiaceta, Paris, France, a corporation of France

No Drawing. Application December 2, 1955  
Serial No. 550,782

Claims priority, application France December 8, 1954

19 Claims. (Cl. 8—24)

This invention relates to the dyeing of mixed textile materials and more particularly to the level dyeing of textile materials containing polyacrylonitrile fibres (as herein defined) and cellulose derivative fibres, with water-soluble dyestuffs, acid dyes, direct dyes and soluble dyes for cellulose acetate.

By "polyacrylonitrile fibres" are meant those produced from polyacrylonitrile or co-polymers of acrylonitrile with other polymerisable monomers containing at least 85% of acrylonitrile in their molecule, or from mixtures of these polymers with other vinyl polymers. Specific fibres of these types are those made from (1) polyacrylonitrile; (2) co-polymers of acrylonitrile with vinyl chloride, vinyl acetate, vinylidene chloride, vinylidene cyanide, methacrylonitrile, acrylic and methacrylic acids and esters and vinylpyridine; the mixtures of these polymers and co-polymers with one another or with vinyl polymers, such as polyvinyl alcohol, chloride or acetate, polymers of vinylidene chloride or vinylidene cyanide, of methacrylonitrile, acrylic and methacrylic acids and esters, of styrene, of vinylpyridine, or the co-polymers based on these products. By "cellulose derivatives" are meant cellulose esters or ethers, e.g. cellulose acetate, cellulose acetobutyrate, ethyl cellulose and benzyl cellulose.

There are generally employed for dyeing polyacrylonitrile fibres either water-insoluble dyestuffs or certain water-soluble dyestuffs specially prepared for dyeing cellulose derivative materials. However, where these dyestuffs are applied to textile articles containing both cellulose derivative fibres and polyacrylonitrile fibres, their affinity for the different fibres is so different that they dye almost exclusively the cellulose derivative fibres. It has heretofore been impossible therefore to effect by the known processes a level dyeing of these two types of fibres when they are mixed in a textile material.

It is known that polyacrylonitrile fibres can be dyed by means of water-soluble dyes in the presence of cuprous salts [Rayon and Synthetic Textiles, 31, 35 (1950); Chemical and Engineering News, 28, 4268 (1950)], but this process is not suitable for dyeing mixtures of fibres containing both polyacrylonitrile fibres and other fibres.

According to the present invention a process for the level dyeing of textile materials containing both cellulose derivative fibres and polyacrylonitrile fibres comprises applying to or incorporating in the cellulose derivative fibres a colourless organic nitrogenous compound having an affinity thereto, and simultaneously or subsequently dyeing the textile materials with water-soluble dyestuffs in the presence of cuprous ions.

The textile materials may be in any form, e.g. filaments, fibres, loose fibre, cabled yarns, union yarns, staple fibre yarns, tows, slivers, woven or knitted fabrics, or pre-formed textile garments or the like. The water-soluble dyestuffs may be acid dyes, direct dyes or water-soluble dyes for cellulose acetate.

The affinity of a nitrogenous organic compound for a textile material is defined by the extent to which the compound is extracted by the said textile material from an aqueous bath in which it is present in the form of a so-

2

lution (true or colloidal), an emulsion or a suspension. In practice, a compound may be regarded as having an affinity for cellulose derivative fibres when, for example, 20 grammes of cellulose derivative fibres present in an aqueous bath containing 1 g./litre of the compound at 80° C. extract and retain at least 25% of the compound from the bath. Products suitable for carrying out the present invention are, for example, saturated heterocyclic compounds having 3 to 7 members in the ring, including a single nitrogen atom, cycloaliphatic amines, amides obtained by condensation of aliphatic monoacids, the chain of which contains at least 12 carbon atoms, with a polymethylene diamine, and the complexes of these various compounds. There may be mentioned, for example, bis - 4:4' - (cyanoethylamino)dicyclohexylmethane, cyanoethyl - spirocyclohexyl - ethylene - imine, piperidine, bis - 4:4' - (monoaminopropylamino)dicyclohexylmethane, cyanoethylaminocyclohexane, cyanoethylaminoethylcyclohexane and cyanomethylhexamethylene-imine, the complexes of these products, in particular the formaldehyde-bisulphite complexes and the monoacylamides of polymethylenediamines. These compounds may, if desired, be previously introduced in known manner into the cellulose derivatives before or during their shaping in the form of filaments. Mixed textile materials containing both cellulose derivative fibres containing these compounds and polyacrylonitrile fibres constitute novel textile materials capable of being uniformly dyed with water-soluble dyestuffs in the presence of cuprous ions.

When the nitrogenous compounds are applied by pre-treatment of the cellulose derivatives, the textile material may be treated, for example, by means of a bath containing from 2% to 15% of the nitrogenous compound, calculated on the weight of the said textile material, depending upon the desired depth of dyeing. From 0.2 to 1 g. per litre of a wetting agent may be added to this bath if desired. The temperature of the pre-treatment may vary from 50° to 100° C. and its optimum duration will depend upon the temperature and can readily be determined by simple tests. The dyeing of the pre-treated textile material may then be carried out in one or two baths, as required. It is also possible to introduce the nitrogenous compound into the dyeing bath containing the desired content of dyestuff or dyestuffs for producing the desired depth of dyeing and a sufficient quantity of acid to bring the pH of the bath to about 3-4; the said bath also contains, or there may subsequently be added thereto, from 2% to 10% of cupric sulphate and from 0.8% to 4% of an appropriate reducing agent (e.g. metallic copper) for reducing the copper sulphate to the cuprous state. If desired, from 0.2 g. to 1 g. per litre of an acid-resisting wetting agent may also be added.

The process according to the invention affords the great advantage of permitting level dyeing in a single bath of textile materials containing different fibres as aforesaid and the dyeings obtained have excellent fastness.

The following examples will serve to illustrate the invention but are not to be regarded as limiting it in any way; the percentages are expressed by weight in relation to the fabric, and the dyestuffs are cited with reference either to "Colour Index" (C.I.) or to "Technical Manual and Year Book of the American Association of Textile Chemists and Colorists" (prototype number: Pr.).

### Example I

A fabric containing both cellulose acetate threads and polyacrylonitrile threads is immersed in 50 times its weight of a bath containing:

10% of formaldehyde-bisulphite complex of bis-4:4'-(cyanoethylamino)-dicyclohexylmethane, 0.2 g. per litre of a wetting agent.

## 3

The fabric is then rinsed and introduced into 50 times its weight of a bath containing:

5% of Anthraquinone Blue SWF, 150% concentration (Pr. 12),  
0.6% of Rocelline S (C.I. 176),  
3 cc. per litre of acetic acid.

After an hour's treatment at boiling point, there are added to the bath:

10% of copper sulphate (pentahydrate),  
4% of sodium formaldehyde sulphoxylate,

and the dyeing is continued for 30 minutes at boiling point in this bath.

The fabric is rinsed and then immersed for 10 minutes in a bath at 40° C. containing 0.2 g. per litre of a condensate of ethylene oxide and oleocetyl alcohol.

A royal blue fabric of very level appearance is obtained.

## Example II

The same fabric as in Example I, having undergone the same pre-treatment, is dipped into 50 times its weight of a bath containing:

0.1% of Anthraquinone Blue SWF, 150% concentration (Pr. 12),  
0.6% of metanil yellow (C.I. 138),  
0.25% of Rocelline S (C.I. 176),  
3 cc. per litre of acetic acid.

After boiling for one hour, there are added to the bath:

2% of copper sulphate (pentahydrate),  
0.08% of hydroxylamine sulphate,

and the dyeing is continued for 30 minutes at boiling point.

The fabric is thoroughly rinsed and immersed for 10 minutes in a bath at 40° C. containing 0.2 g. per litre of a condensate of ethylene oxide and an alkyl phenol.

## Example III

Discontinuous polyacrylonitrile fibres and discontinuous ethyl cellulose fibres, the latter containing 8% of its weight of cyanoethylspirocyclohexyl-ethylene-imine introduced during the manufacture of the fibres, are intimately mixed in equal proportions and spun together. The yarns and fabrics obtained with this mixed material may be dyed with a very satisfactory level effect by acid or soluble dyestuffs in the presence of cuprous ions.

## Example IV

A fabric obtained from yarns formed of intimately mixed discontinuous acrylonitrile and vinyl chloride co-polymer fibres and discontinuous cellulose acetate fibres is introduced into 50 times its weight of a bath containing:

10% of formaldehyde-bisulphite complex of bis-4:4'-(cyanoethylamino)dicyclohexylmethane,  
5% of Anthraquinone Blue SWF (Pr. 12),  
0.2 g. per litre of a wetting agent.

After boiling for 30 minutes there are added:

3 cc. per litre of acetic acid.

The boiling is continued for 30 more minutes, whereafter there are introduced:

10% of copper sulphate (pentahydrate),  
4% of hydroxylamine sulphate.

The boiling is maintained for 30 more minutes and the article is rinsed, and dried. A very level blue dyeing is obtained.

## 4

## Example V

The same fabric as in Example I, having undergone the same treatment with the formaldehyde-bisulphite complex of bis-4:4'-(cyanoethylamino)dicyclohexylmethane, is dipped into 50 times its weight of a bath containing:

1% of "jaune Solacet solide GS" (commercial water-soluble dyestuff for cellulose acetate),  
1% of "bleu Solacet solide 2BS" (commercial water-soluble dyestuff for cellulose acetate),  
3 cc. per litre of acetic acid.

After treatment for 1½ hours at boiling point, there are added to the bath:

10% of copper sulphate (pentahydrate),  
4% of hydroxylamine sulphate,

and the dyeing is continued for 30 minutes at boiling point.

The article is thoroughly rinsed and a very level green-dyed fabric is obtained.

## Example VI

The same fabric as in Example I is introduced into 50 times its weight of a bath containing:

5% of formaldehyde-bisulphite complex of bis-4:4'-(cyanoethylamino)dicyclohexylmethane,  
0.2 g. per litre of a wetting agent.

After treatment for one hour at 80° C. the fabric is rinsed and then introduced into 50 times its weight of a bath containing:

5% of Anthraquinone Blue SWF, 150% concentration (Pr. 12),  
0.6% of Rocelline S (C.I. 176),  
0.2 g. per litre of a wetting agent,  
3 cc. per litre of acetic acid,  
10% of copper sulphate (pentahydrate),  
4% of hydroxylamine sulphate.

The dyeing is carried out in this bath for one hour at boiling point. The article is thoroughly rinsed and a very level royal blue fabric is obtained.

## Example VII

The same fabric as in Example I is introduced into 50 times its weight of a bath containing:

5% of the monamide obtained by the condensation of stearic acid and trimethylene-diamine,  
0.2 g. per litre of a wetting agent.

After treatment for one hour at 80° C. the fabric is rinsed and then introduced into 50 times its weight of a bath containing:

1.8% of Orange II (C.I. 151),  
0.35% of Rocelline S (C.I. 176),  
1.15% of Anthraquinone Blue SWF, 150% concentration (Pr. 12).

After treatment for one hour at boiling point, there are added to the bath:

10% of copper sulphate (pentahydrate),  
4% of hydroxylamine sulphate,

and the dyeing is continued for 30 minutes at boiling point. The article is thoroughly rinsed and a very level brown fabric is obtained.

## Example VIII

The same fabric as in Example I is introduced into 50 times its weight of a bath containing:

5% of the formaldehyde-bisulphite complex of bis-4:4'-(cyanoethylamino)dicyclohexylmethane,  
0.2 g. per litre of a wetting agent.

After treatment for one hour at 80° C. the fabric is rinsed and then introduced into 50 times its weight of a bath containing:

0.1% of Anthraquinone Blue SWF, 150% concentration (Pr. 12),  
0.25% of Rocelline S (C.I. 176),  
0.6% of metanil yellow (C.I. 138),  
2% of copper sulphate (pentahydrate),  
A copper plate,  
3 cc. per litre of acetic acid.

The dyeing is carried out in this bath for one hour at boiling point. The article is thoroughly rinsed and a very level grey-green fabric is obtained.

I claim:

1. A process for the level dyeing of textile materials containing both fibres of a cellulose derivative selected from the class consisting of the water-insoluble esters and ethers of cellulose and fibres of an acrylonitrile polymer selected from the class consisting of acrylonitrile homopolymer and copolymers of acrylonitrile with other vinyl compounds copolymerisable therewith, which copolymers contain at least 85% of acrylonitrile units, which comprises incorporating in said cellulose derivative fibres a colourless organic nitrogenous monomeric compound selected from the group which consists of (1) saturated heterocyclic compounds having 3-7 members in the ring, of which one is a single nitrogen atom, (2) cycloaliphatic amines, (3) amides obtained by the condensation of an aliphatic monocarboxylic acid having at least 12 carbon atoms in the chain with a polymethylene diamine, and (4) complexes of these compounds.

2. Process according to claim 1, wherein there is incorporated in the cellulose derivative fibres a compound selected from the group consisting of bis-4:4'-(cyanoethylamino)-dicyclohexylmethane, its formaldehyde bisulphite complex, cyanoethyl-spirocyclohexyl-ethylene-imine and stearic acid 3-aminopropylamide.

3. Process according to claim 1 wherein the cellulose derivative is cellulose acetate.

4. Process according to claim 3, wherein there is incorporated in the cellulose acetate fibres a compound selected from the group which consists of bis-4:4'-(cyanoethylamino)-dicyclohexylmethane, its formaldehyde bisulphite complex, cyanoethyl-spirocyclohexyl-ethylene-imine and stearic acid 3-aminopropylamide.

5. Process according to claim 3, wherein stearic acid 3-aminopropylamide has been incorporated in the cellulose acetate fibres during their manufacture.

6. Process according to claim 1, which comprises incorporating bis-4:4'-(cyanoethylamino)-dicyclohexylmethane in the textile material by treating the material with an aqueous bath containing 2-15% thereof, based on the weight of the textile material.

7. Process according to claim 6, wherein the textile material contains both cellulose acetate fibres and fibres of the said acrylonitrile polymer.

8. Process according to claim 1, which comprises incorporating the formaldehyde bisulphite complex of

bis-4:4'-(cyanoethylamino)-dicyclohexylmethane in the textile material by treating the material with an aqueous bath containing 2-15% thereof, based on the weight of the textile material.

5 9. Process according to claim 8, wherein the textile material contains both cellulose acetate fibres and fibres of the said acrylonitrile polymer.

10. Process according to claim 1, which comprises incorporating stearic acid 3-aminopropylamide in the textile material by treating the material with an aqueous bath containing 2-15% thereof, based on the weight of the textile material.

11. Process according to claim 10, wherein the textile material contains both cellulose acetate fibres and fibres of the said acrylonitrile polymer.

12. Process according to claim 1, wherein cyanoethyl-spirocyclohexyl-ethylene-imine has been incorporated in the cellulose derivative fibres during their manufacture.

13. Process according to claim 12, wherein the textile material contains both cellulose acetate fibres and fibres of the said acrylonitrile polymer.

14. Process according to claim 1, which comprises dyeing the textile material with a dyebath containing a water-soluble dyestuff, cuprous ions, and 2-15%, by weight of

25 the textile fabric, of bis-4:4'-(cyanoethylamino)-dicyclohexylmethane.

15. Process according to claim 14, wherein the textile material contains both cellulose acetate fibres and fibres of the said acrylonitrile polymer.

30 16. Process according to claim 1, which comprises dyeing the textile material with a dyebath containing a water-soluble dyestuff, cuprous ions, and 2-15%, by weight of the textile fabric, of the formaldehyde bisulphite complex of bis-4:4'-(cyanoethylamino)-dicyclohexylmethane.

17. Process according to claim 16, wherein the textile material contains both cellulose acetate fibres and fibres of the said acrylonitrile polymer.

18. Process according to claim 1, which comprises dyeing the textile material with a dyebath containing a water-soluble dyestuff, cuprous ions, and 2-15%, by weight of the textile fabric, of stearic acid 3-aminopropylamide.

40 19. Process according to claim 18, wherein the textile material contains both cellulose acetate fibres and fibres of the said acrylonitrile polymer.

#### References Cited in the file of this patent

#### UNITED STATES PATENTS

|           |         |       |                |
|-----------|---------|-------|----------------|
| 2,277,829 | Heckert | ----- | Apr. 8, 1941   |
| 2,615,781 | Olpin   | ----- | Oct. 28, 1952  |
| 2,760,841 | Salvin  | ----- | Aug. 28, 1956  |
| 2,775,022 | Davis   | ----- | Dec. 25, 1956  |
| 2,805,465 | Miller  | ----- | Sept. 10, 1957 |

#### OTHER REFERENCES

Technical Bulletin by du Pont, vol. 7, No. 1, March 1951, pp. 45, 46 and 52.